# EUROPEAN PATENT SPECIFICATION

(11) **EP 3 239 344 B1**
(45) Date of publication and mention of the grant of the patent: **20.10.2021**
(21) Application number: 15873672.8
(22) Date of filing: 24.12.2015
(51) Int. Cl.: B22D 11/124, B22D 11/16, B22D 11/055, C22C 38/00, C22C 38/58, C22C 38/42, C22C 38/04, B22D 11/22, C22C 38/44, C21D 6/00, C22C 38/02, C22C 38/34, C22C 38/46, C22C 38/48, C22C 38/50

(54) **METHOD FOR PRODUCING A LEAN DUPLEX STAINLESS STEEL**
VERFAHREN ZUR HERSTELLUNG EINES LEAN DUPLEX EDELSTAHLS
PROCÉDÉ DE PRODUCTION D'UN ACIER INOXYDABLE LEAN DUPLEX

(30) Priority: 26.12.2014 KR 20140191170
(43) Date of publication of application: 01.11.2017
(73) Proprietor: POSCO, Pohang-si, Gyeongsangbuk-do 37859 (KR)
(72) Inventor: CHOI, Jeom Yong, Pohang-si Gyeongsangbuk-do 37671 (KR)
(74) Representative: Potter Clarkson
(86) International application number: PCT/KR2015/014235
(87) International publication number: WO 2016/105145

(56) References cited:
- EP-A1- 1 715 073
- EP-A1- 2 246 453
- EP-A1- 2 699 704
- WO-A1-96/24452
- WO-A1-2013/081422
- CN-A- 102 634 740
- CN-A- 104 131 237
- JP-A- 2005 154 890
- JP-A- 2010 196 103
- KR-A- 20010 073 236
- KR-A- 20120 016 369
- KR-A- 20130 060 658
- KR-A- 20130 125 071
- KR-A- 20140 052 079
- KR-A- 20140 080 347
- KR-A- 20140 080 347
- KR-A- 20140 082 491
- KR-A- 20140 082 491
- KR-A- 20140 084 721
- None

## Description

### TECHNICAL FIELD

The present invention relates to lean duplex stainless steel having a ferritic-austenitic structure and a method for producing the same.

### BACKGROUND ART

In general, the austenitic stainless steel with good workability and corrosion resistance contains iron (Fe) as a base metal and chromium (Cr) and nickel (Ni) as main raw materials, and has been developed as a variety of steel to meet various applications by adding other elements such as molybdenum (Mo) and copper (Cu).

300 series stainless steel, which is excellent in corrosion resistance and workability, contains expensive raw materials such as Ni and Mo, and thus, as an alternative to this, 200- and 400-series stainless steels have been discussed. However, 200-series and 400-series stainless steels have disadvantages respectively in that their formability and corrosion resistance do not reach to 300-series stainless steel.

On the other hand, the duplex stainless steel in which an austenite phase and a ferrite phase are mixed has all the advantages of the austenitic stainless steel and the ferritic stainless steel, and thus, to date, various types of duplex stainless steels have been developed.

In addition, in recent years, in order to compensate for the shortcoming of price competitiveness, there is an increasing interest in lean duplex stainless steels, in which high-cost alloying elements such as Ni and Mo contained in the duplex stainless steels are eliminated and low-cost alloying elements are added to further enhance cost advantages.

However, such lean duplex stainless steels have a disadvantage in that they have a poor hot workability depending on the difference in strength between the ferrite phase and the austenite phase, resulting in a large number of surface cracks and edge cracks.

In addition, if alloy elements whose components were adjusted for lean duplex stainless steel are processed according to a conventional and general continuous casting process, a large number of pores are generated inside the slab due to the difference in nitrogen solubility when solidified from a liquid phase to a solid phase. These internal pores are the cause of generating a large number of defects on the surface of the product during the reheating and hot rolling processes which are subsequent processes, and also causes the disadvantage of generating a large number of cracks on the edge of the hot rolled coil.

EP 2699704 A1 discloses a ferrite-austenitic lean duplex stainless steel having good formability, good weldability and high elongation. The C+N content lies in the range 0.17 wt% - 0.295 wt% and heat treatment results in a microstructure that is 45-75% austensite with the remainder being ferrite. The measured M_{d30} temperature of the steel is adjusted to be between 0 and 50°C in order to utilise transformation-induced plasticity in improving formability.

EP 1715073 A1 discloses an austenitic-ferrite stainless steel that exhibits high formability and punch stretchability; and crevice corrosion resistance. The stainless steel has a mainly austenite-ferrite microstructure and consists essentially of 0.2% or less C, 4% or less Si, 12% or less Mn, 0.1% or less P, 0.03% or less S, 15-35% Cr, 3% or less Ni and 0.05 to 0.6% N with the austenite phase being adjusted to be from 10 to 85% by volume and the total of (C+N) in the austenite phase being in the range 0.16 - 2%.

WO2013/081422 A1 discloses a lean duplex stainless steel and a preparation method thereof. The lean duplex stainless steel comprises 0.08% or less of C, 0.2 - 3.0% or less of Si, 2 - 4% of Mn, 19 - 23% of Cr, 0.3 - 2.5% of Ni, 0.2 - 0.3% of N, 0.5 - 2.5% of Cu and the balance Fe and inevitable impurities. The preparation method involves preparing a thin sheet by allowing molten steel to pass between a pair of casting rolls wherein nitrogen exceeding the nitrogen solubility limit in the molten steel is discharged through the casting rolls.

### DISCLOSURE

### TECHNICAL PROBLEM

The present invention provides lean duplex stainless steel capable of ensuring excellent elongation and corrosion resistance and a method of manufacturing the same, by controlling the content of alloy components to reduce costs and also satisfactorily control the stacking fault energy value present in the lean-duplex stainless steel.

Also, the present invention provides a lean duplex stainless steel capable of ensuring excellent elongation and corrosion resistance and a method of manufacturing the same, by satisfactorily controlling the value of the critical strain for strain induced martensite formation.

Further, the present invention provides a lean duplex stainless steel capable of solving the problem of massive release of nitrogen gas due to a sharp reduction in nitrogen solubility during solidification from a liquid phase to a solid phase in casting, and a method of manufacturing the same.

### TECHNICAL SOLUTION

A method according to the invention of manufacturing a ferrite-austenitic lean duplex stainless steel comprises preparing a molten steel including, by weight, C: 0.08% or less excluding 0%, Si: 0.2 to 3.0%, Mn: 2 to 4%, Cr: 18 to 24%, Ni: 0.2 to 2.5%, Cu: 0.2 to 2.5%, N: 0.15 to 0.32%, optionally at least one of W: 0.1 to 1.0% and Mo: 0.1 to 1.0%, optionally at least one of Ti: 0.001 to 0.1%, Nb: 0.001 to 0.05%, and V: 0.001 to 0.15%, balance Fe and the other unavoidable impurities, continuous casting the stainless steel, with additional hot rolling annealing or cold rolling annealing at 900 to 1200°C, wherein the stainless steel is annealing heat treated so that the stacking fault energy (SFE) value of the austenite phase represented by the following Formula 2 is 19 to 37 mJ/m² and the range of the value of the critical strain for strain induced martensite formation is 0.1 to 0.25, wherein the value of the critical strain is measured from the inflection point of the stress-strain curve and obtained by taking a specimen with ASTM sub-size standard in parallel with the rolling direction in cold-rolled annealed material, and a tensile test is performed at 20 to 25°C in a strain rate of 1.0 × 10⁻³/s using the tensile tester until the material is broken; $\begin{matrix}SFE = 25.7 + 1.59 \times Ni / \left[K\left(Ni\right)-K\left(Ni\right)\times V\left(γ\right)+V\left(γ\right)\right] + 0.795 \times Cu / \left[K\left(Cu\right)-K\left(Cu\right)\times V\left(γ\right)+V\left(γ\right)\right] - \\ 0.85 \times Cr / \left[K\left(Cr\right)-K\left(Cr\right)\times V\left(γ\right)+V\left(γ\right)\right] + 0.001 \times {\left(Cr/\left[K\left(Cr\right)-K\left(Cr\right)\times V\left(γ\right)+V\left(γ\right)\right]\right)}^{2} + 38.2 \times {\left(N/\left[\begin{matrix}K \left(N\right) - \\ K \left(N\right) \times V \left(γ\right) + V \left(γ\right)\end{matrix}\right]\right)}^{0.5} \\ - 2.8 \times Si / \left[K\left(Si\right)-K\left(Si\right)\times V\left(γ\right)+V\left(γ\right)\right] - 1.34 \times Mn / \left[\begin{matrix}K \left(Mn\right) - \\ K \left(Mn\right) \times V \left(γ\right) + V \left(γ\right)\end{matrix}\right] \\ + 0.06 \times {\left(Mn/\left[K\left(Mn\right)-K\left(Mn\right)\times V\left(γ\right)+V\left(γ\right)\right]\right)}^{2}\end{matrix}$
wherein the continuous casting includes temporarily storing the molten steel in the tundish while maintaining the temperature of the molten steel at the temperature higher than the theoretical solidification temperature by 10 to 50 °C, primarily cooling the molten steel by injecting the molten steel in the tundish into the mold and passing the molten steel through the mold while maintaining a cooling rate of 500 to 1500 °C/min, secondarily cooling the molten steel having the solidified shell formed by the primary cooling process by spraying cooling water of 0.25 to 0.35 L/Kg on the molten steel having the formed solidified shell while drawing it into a segment and passing through, and tertiary cooling is performed by spraying the cooling water of 100 to 125 L/kg · min on the surface of the cast-slab in the range of the surface temperature of the cast-slab being drawn of 1100 to 1200 °C wherein the cooling water is mixed with air such that the ratio of air to cooling water air/cooling water is 1.0 to 1.2; and
wherein Ni, Cu, Cr, N, Si and Mn refer to the overall content (wt.%) of respective constituent elements respectively, and K(x) is represented by the following formula 3 as the distribution coefficient of respective constituent element (x) measured using Fe-EPMA and FE-TEM, and V(γ) is the fraction of the austenite phase and lies in the range of 0.45 to 0.75; $K \left(x\right) = \left[content of element x in ferrite phase\right] / \left[content of element x in austenic phase\right]$
wherein regarding the K(x), K(Cr) = 1.16, K(Ni) = 0.57, K(Mn) = 0.73, and K(Cu) = 0.64, and K(N) and K(Si) have the following values depending on the content in wt.% of N and Si:
   when N is 0.2 to 0.32%, K(N) = 0.15;
   when N < 0.2%, K(N) = 0.25;
   when Si ≤ 1.5%, K(Si) = 2.76-0.96×Si; and
   when Si > 1.5%, K(Si) = 1.4, and
wherein the elongation of the stainless steel is 45% or more, wherein the stainless steel includes, by weight, C: 0.08% or less excluding 0%, Si: 0.2 to 3.0%, Mn: 2 to 4%, Cr: 18 to 24%, Ni: 0.2 to 2.5%, Cu: 0.2 to 2.5%, N: 0.15 to 0.32%, optionally at least one of W: 0.1 to 1.0% and Mo: 0.1 to 1.0%, optionally at least one of Ti: 0.001 to 0.1%, Nb: 0.001 to 0.05%, and V: 0.001 to 0.15%, balance Fe and the other unavoidable impurities, wherein the critical strain for strain induced martensite formation is measured by way of a tensile test as defined herein, , and wherein the lean duplex stainless steel is formed as austenite phases of 45 to 75% and ferrite phases of 25 to 55% by volume fraction, the sum of the austenite and ferrite phases equalling 100%.

In particular, the process of treating the molten steel to form the stainless steel comprises temporarily storing the molten steel in the tundish while maintaining the temperature of the molten steel at the temperature higher than the theoretical solidification temperature by 10 to 50 °C; primarily cooling the molten steel by injecting the molten steel in the tundish into the mold and passing the molten steel through the mold while maintaining a cooling rate of 500 to 1500 °C/min; and secondarily cooling the molten steel having a solidified shell formed by the primary cooling process while drawing it into a segment and passing through.

At this time, in the secondary cooling process, it is required to spray cooling water of 0.25 to 0.35 L/kg on the molten steel having the formed solidified shell.

Further, the method comprises tertiarily cooling, after the secondary cooling process, by spraying cooling water of 100 to 125 L/kg · min on the surface of the cast-slab in the range of the surface temperature of the cast-slab being drawn of 1100 to 1200 °C wherein the cooling water is mixed with air such that the ratio of air to cooling water is 1.0 to 1.2

Meanwhile, a process of treating the molten steel (not forming part of the invention) to form the stainless steel may comprise producing a strip by solidifying the molten steel while passing it between a pair of casting rolls wherein nitrogen contained in the molten steel in the process of producing the strip and exceeding a nitrogen solubility limit can be discharged through the casting roll to the outside of the solidified shell.

At this time, in such a process of producing the strip, it is preferable to use a casting roll, in which a gas discharge channel is formed in the circumferential direction on the outer peripheral surface, as at least one of a pair of casting rolls

In addition, the gas discharge channel formed in the casting roll used in the process of producing the strip has a width of 50 to 500 *µ*m and a depth of 50 to 300 *µ*m, a plurality of gas discharge channels is formed in the casting roll, the gap between adjacent gas discharge channels is 100 to 1000 *µ*m and unevennesses of 15 to 25 *µ*m are formed on the surface of the casting roll.

### ADVANTAGEOUS EFFECTS

According to the embodiment of the present invention, it is possible to save resources and significantly reduce the cost of raw materials by controlling the contents of the alloy components of Ni, Si and Cu which are high-priced elements, and in particular it is sufficiently usable as an alternative to the 200 and 300 series (STS 304, 316) used for molding, by ensuring corrosion resistance and excellent elongation at the same level or higher compared to STS 304.

Further, the continuous casting of the alloying elements according to the invention permits control of the temperature of the molten steel and the cooling rate to suppress the pinholes generated inside the cast-slab.

Further, in the case of strip casting of the alloying element, according to a method which is not part of the present invention, the generation of the internal pores and the occurrence of surface defects can be prevented by smoothly inducing the discharge of the nitrogen gas generated when solidified from a liquid phase to a solid phase, through the improvement of the casting roll.

### BRIEF DESCRIPTION OF THE DRAWINGS

FIG. 1 is a view showing a value of critical strain for strain induced martensite phase formation as stress-strain curves of an inventive steel according to an embodiment of the present invention and a comparative steel.
FIGs. 2a and 2b are photographs showing the formation of strain induced martensite phases as representative transmission electron microscope photographs of an inventive steel according to an embodiment of the present invention and a comparative steel.
FIG. 3 is a graph showing the relationship between the elongation and the value of critical strain for strain induced martensite phase formation.
FIG. 4 is a schematic view illustrating a manufacturing process of continuous casting method of the lean duplex stainless steel according to an embodiment of the present invention.
FIG. 5 is a schematic view illustrating a manufacturing process of strip casting method of the lean duplex stainless steel that is not part of the present invention.
FIG. 6 is a photomicrograph illustrating a casting roll required in a manufacturing process of strip casting method of the lean-duplex stainless steel that is not part of the present invention.
FIG. 7 is a photograph of the structure of the comparative material I and the inventive material A.
FIG. 8 is a photograph of surface defects of the comparative material H.
FIG. 9 is a photograph of surface defects of the comparative material F.

### BEST MODE FOR THE INVENTION

Hereinafter, embodiments of the present invention will be described in more detail with reference to the accompanying drawings. However, the present invention is only limited by the scope of the appended claim.

FIG. 1 is a view showing a value of critical strain for strain induced martensite formation as stress-strain curves of the inventive steel according to an embodiment of the present invention and the comparative steel.

The present invention relates to lean duplex stainless steel having two-phase structures formed of a ferrite phase and an austenite phase comprising, by weight (unless otherwise specified below, the content of the ingredients is % by weight), C: 0.08% or less (excluding 0%), Si: 0.2 to 3.0%, Mn: 2 to 4%, Cr: 18 to 24%, Ni: 0.2 to 2.5%, N: 0.15 to 0.32 %, Cu: 0.2 to 2.5%, N: 0.15 to 0.32%, at least one of W: 0.1 to 1.0% and Mo: 0.1 to 1.0%, at least one of Ti: 0.001 to 0.1%, Nb: 0.001 to 0.05%, and V: 0.001 to 0.15%, balance Fe, and the other unavoidable impurities.

C is an element for forming an austenite phase and is an effective element for increasing the strength of a material by solid solution strengthening. However, since C, when added excessively, easily bonds with carbide-forming elements such as Cr, which is effective for corrosion resistance at the ferrite-austenite phase boundary, thereby reducing the Cr content around the grain boundary and thus reducing the corrosion resistance, C is added in a range of more than 0% to 0.08% or less in order to maximize the corrosion resistance.

Si is partially added for the deoxidation effect, is an element for forming a ferrite phase and is an element which is concentrated on the ferrite phase during the annealing heat treatment. Therefore, 0.2% or more should be added to ensure a proper ferrite phase fraction. However, the excessive addition of Si exceeding 3.0% increases the hardness of the ferrite phase drastically and thus affects the lowering of the elongation of the two-phase steel, and also makes it difficult to ensure the austenite phase for ensuring sufficient elongation. Further, Si, when being added excessively, lowers the slag fluidity at the time of steelmaking and bonds with oxygen to form inclusions, thereby deteriorating the corrosion resistance. Therefore, the content of Si is limited to 0.2 to 3.0%.

Mn is an element that increases the deoxidizing agent and nitrogen solubility, and is an austenite phase forming element and can be used for replacing expensive Ni. When Mn is added in a large amount, excessive Mn is effective for solubility of nitrogen, but combines with S in the steel to form MnS, thereby deteriorating the corrosion resistance. Therefore, when its content exceeds 4%, it becomes difficult to ensure the corrosion resistance of the level of 304 steel. In addition, when the content of Mn is less than 2%, even if Ni, Cu, N and the like which are the austenite phase forming elements are controlled, it is difficult to ensure a proper austenite phase fraction, and the solubility of N to be added is low and thus sufficient solution of nitrogen at normal pressure cannot be obtained. Therefore, the content of Mn is limited to 2 to 4%.

Cr is an element for stabilizing the ferrite phase together with Si and plays a major role in ensuring the ferrite phase of the two-phase stainless steel, as well as it is an essential element for ensuring corrosion resistance. When the Cr content is increased, the corrosion resistance increases, but in order to maintain the phase fraction, the content of expensive Ni or other austenite phase forming elements must be increased. Accordingly, in order to ensure corrosion resistance equal to or higher than that of 304 steel while maintaining the phase fraction of the two-phase stainless steel, the content of Cr is limited to 18 to 24%.

Ni is an element for stabilizing the austenite phase together with Mn, Cu and N, and plays a main role in ensuring the austenite phase of the duplex stainless steel. By increasing Mn and N, which are other austenite phase forming elements, instead of maximally decreasing the content of expensive Ni for cost reduction, it is possible to sufficiently maintain the phase fraction balance that can be influenced by the reduction of Ni. However, in order to suppress the formation of strain induced martensite phase which occurs during the cold processing and accordingly to ensure sufficient austenite phase stability, it is necessary to add at least 0.2%. When a large amount of Ni is added, it is difficult to ensure a proper austenite phase fraction because the fraction of the austenite phase increases and in particular, it is difficult to ensure competitiveness compared to 304 steel due to an increase in the manufacturing cost of products by expensive Ni. Therefore, the content of Ni is limited to 0.2 to 2.5%.

N is an element that contributes greatly to the stabilization of the austenite phase together with Ni in the duplex stainless steel and is one of the elements which is mostly concentrated on the austenite phase due to the high diffusion rate on the solid phase during the annealing heat treatment. Therefore, the increase of the N content can incidentally induce an increase in corrosion resistance and an increase in strength. However, the solubility of N varies depending on the content of Mn added. When the N content exceeds 0.32% in the range of Mn of the present invention, it is difficult to stably produce steel due to generation of surface defects such as blow holes or pinholes during casting due to excessive nitrogen solubility. On the other hand, N is added in the amount of 0.15% or more in order to ensure the corrosion resistance of the level of 304 steel. If the content of N is too low, it becomes difficult to ensure a proper phase fraction. Therefore, the content of N is limited to 0.15 to 0.32%.

Cu is an element for stabilizing the austenite phase together with Mn, Ni and N, and it is desirable that the content of Cu, which plays the same role as Ni, should be minimized for cost reduction. However, it is preferable to add at least 0.2% in order to ensure the stability of the austenite phase sufficient to suppress the excessive formation of the strain induced martensite phase occurring during cold processing. On the other hand, if the content of Cu exceeds 2.5%, it becomes difficult to process the product due to hot brittleness. Therefore, the content of Cu is adjusted to 0.2 to 2.5%.

W and Mo are optional elements for forming the austenite phase and elements for improving corrosion resistance, and are elements that promote the formation of an intermetallic compound at 700 to 1000 °C during heat treatment, resulting in deterioration of corrosion resistance and mechanical properties. When the content of W and Mo exceeds 1% respectively, an intermetallic compound is formed, which may lead to a rapid decrease in corrosion resistance and particularly in elongation. In addition, 0.1% or more can be added in order to exhibit the effect of improving the corrosion resistance. Therefore, the content of W and Mo is limited to 0.1 to 1.0% respectively, and at least one of W and Mo is included.

Ti, Nb, and V are optional elements that react with nitrogen to form nitrides, and they are crystallized as TiN, NbN, and VN respectively in the molten steel and act as nucleation sites on the ferrite phase during solidification, so that sufficient solidification can proceed even when the cooling rate is increased, thereby suppressing the breakage of the slab. In addition, these elements are sufficiently dissolved during the manufacturing process, i.e., reheating or hot rolling, and react with carbon and nitrogen during cooling to form carbonitride and thus inhibit the formation of Cr carbide, thereby contributing to improvement of corrosion resistance. In particular, they are elements that inhibit the formation of Cr carbide in the heat affected zone during welding. When each of these elements is excessively added, that is, when Ti is more than 0.1%, Nb is more than 0.05%, and V is more than 0.15%, these crystals in the solidification form large clusters and cause clogging phenomenon that block the casting nozzle and further, when existing in the surface layer portion of the slab, they act as the cause of defects during rolling and breakage during processing. In addition, since most of these are expensive alloying elements, the addition of a large amount causes an increase in manufacturing cost. Therefore, the range of Ti is limited to 0.001 to 0.1%; the range of Nb is limited to 0.001 to 0.05%, the range of V is limited to 0.001 to 0.15%, and at least one of Ti, Nb and V is included.

Meanwhile, the present invention maintains elongation and corrosion resistance excellently by controlling the content of the alloy elements, the distribution coefficient and the phase fraction to control the stacking fault energy

The following formula 1 is a formula for deriving the stacking fault energy by utilizing the content of all components in the alloy. $SFE = 25.7 + 1.59 \left(Ni+0.5Cu\right) - 0.85 Cr + 0.001 {Cr}^{2} + 38.2 {N}^{0.5} - 2.8 Si - 1.34 Mn + 0.06 {Mn}^{2} -$ wherein Cr, Ni, Cu, Si, Mn, and N mean the overall content (wt.%) of respective constituent elements.

However, the applicants of the present invention have found that as a result of measuring and calculating the stacking fault energies of the inventive steel by various methods, it is more accurate to predict the properties of the alloy by calculating the stacking fault energy while utilizing the content of the components of the austenite structure rather than calculating it using only the content of the components of the overall alloy composition as in formula 1. The applicants of the present invention have found that for this purpose, calculating the stacking fault energy taking into account the interstitial distribution coefficient of the alloying elements rather than calculating the stacking fault energy by using only the component content of the overall alloy composition can obtain a more accurate approximation of the actually measured stacking fault energy value.

Therefore, the applicants of the present invention have made the following formula 2 by supplementing formula 1 above so as to deduce the stacking fault energy of the austenite phase by utilizing the distribution coefficient of the austenite phase. $\begin{matrix}SFE = 25.7 + 1.59 \times Ni / \left[K\left(Ni\right)-K\left(Ni\right)\times V\left(γ\right)+V\left(γ\right)\right] + 0.795 \times Cu / \left[K\left(Cu\right)-K\left(Cu\right)\times V\left(γ\right)+V\left(γ\right)\right] - \\ 0.85 \times Cr / \left[K\left(Cr\right)-K\left(Cr\right)\times V\left(γ\right)+V\left(γ\right)\right] + 0.001 \times {\left(Cr/\left[K\left(Cr\right)-K\left(Cr\right)\times V\left(γ\right)+V\left(γ\right)\right]\right)}^{2} + 38.2 \times {\left(N/\left[\begin{matrix}K \left(N\right) - \\ K \left(N\right) \times V \left(γ\right) + V \left(γ\right)\end{matrix}\right]\right)}^{0.5} \\ - 2.8 \times Si / \left[K\left(Si\right)-K\left(Si\right)\times V\left(γ\right)+V\left(γ\right)\right] - 1.34 \times Mn / \left[\begin{matrix}K \left(Mn\right) - \\ K \left(Mn\right) \times V \left(γ\right) + V \left(γ\right)\end{matrix}\right] \\ + 0.06 \times {\left(Mn/\left[K\left(Mn\right)-K\left(Mn\right)\times V\left(γ\right)+V\left(γ\right)\right]\right)}^{2}\end{matrix}$ wherein Ni, Cu, Cr, N, Si and Mn refer to the overall content (wt.%) of respective constituent elements, and K(x) is represented by the following Formula 3 as the distribution coefficient of respective constituent element (x). $K \left(x\right) = \left[content of element x in ferrite phase\right] / \left[content of element x in austenite phase\right]$

The applicants of the present invention measured the distribution coefficients for respective alloying elements in various annealing conditions and alloy systems by using Fe-EPMA and FE-TEM which are more accurate than EDAX analysis by conventional scanning electron microscopy. At this time, it was confirmed that the distribution coefficients for most of the measured alloying elements are not changed depending on the change of temperature at 900 to 1200 °C, which is the temperature range of hot rolling annealing or cold rolling annealing.

That is, regarding the K(x) values, K(Cr) = 1.16, K(Ni) = 0.57, K(Mn) = 0.73, and K(Cu) = 0.64, and it was confirmed that K(N) and K(Si) vary depending on the content of N and Si (wt.%). However, when N: 0.2 to 0.32%, K(N) = 0.15, when N < 0.2%, K(N) = 0.25, when Si ≤ 1.5%, K(Si) = 2.76-0.96×Si, and when Si > 1.5, K(Si) = 1.4. At this time, the alloying elements N and Si mean the entire components of the stainless steel. However, in the present embodiment, since N: 0.15 to 0.32%, when N: 0.15 or more and less than 0.2%, K (N) = 0.25 will be applied and when N: 0.2 to 0.32, K (N) = 0.15 will be applied, and since Si: 0.2 to 3.0%, when Si: 0.2 to 1.5%, K(Si) = 2.76-0.96×Si will be applied and when Si: more than 1.5% and 3.0% or less, K(Si) = 1.4 will be applied.

In addition, in the formula 2, V(γ) is the austenite phase fraction, and the austenite phase fraction is defined by the following relation function. $1 = V \left(α\right) + V \left(γ\right)$ wherein V(α) is the ferrite phase fraction, and V(γ) has the range of 0.45 to 0.75.

On the other hand, the reason for limiting the stacking fault energy value of the austenite phase to 19 to 37 mJ/m² is explained below.

The stacking fault energy of the austenite phase is known to control the transformation mechanism of the austenite phase. Typically, the stacking fault energy of the austenite phase in the case of single-phase austenitic stainless steel represents the extent to which the externally applied plastic strain energy contributes to the strain of the austenite phase. Generally, the lower the stacking fault energy, the greater the degree of formation of the strain induced martensite phase that contributes to the work hardening of the steel after formation of the epsilon martensite phase on the austenite phase. If the stacking fault energy is moderate, mechanical twinning is formed in the austenite phase. In the case of moderate stacking fault energies, the strain induced martensite phase is formed at the twinning intersection, so that the applied plastic strain energy causes mechanical phase change and thus transformation from the austenite phase to martensite phase. Therefore, the stainless steel is known to form the strain induced martensite phase in a very broad range, except for difference in the mesophase (the epsilon martensite phase or the mechanical twin). Accordingly, when the stacking fault energy is less than 50 mJ/m², the strain induced martensite phase is formed after the epsilon martensite phase is formed in the austenite phase, or the strain induced martensite phase is formed after the mechanical twin is formed in the austenite phase.

However, it is known that when the stacking fault energy is 50 mJ/m² or more, since the strain proceeds by dislocation movement without formation of the mechanical twin or the epsilon martensite phase, transformation from the austenite phase to the martensite phase does not work well.

On the other hand, it was confirmed that when Formula 1 is applied to deduce the stacking fault energy only from the overall components of the alloy, formation of the strain induced martensite phase is easy when being at 11 mJ/m² or less and thus in the early stage of the strain, rapid work hardening is caused, that is, the strain induced martensite phase is formed, thereby resulting in a sharp decrease in elongation. However, it was confirmed that since the alloying elements distributed to the austenite phase vary depending on the heat treatment or the manufacturing process, the formation behavior of strain induced martensite phases varies in some component systems.

Therefore, the applicants of the present invention corrected the formula as in formula 2 above, taking into account the distribution coefficients of the alloying elements distributed to the austenite phase after various manufacturing processes and heat treatments. As a result, when the calculated stacking fault energy of the austenite phase is less than 19 mJ/m², the epsilon martensite phase is first formed as the medium phase and the martensite phase is formed at the intersection of the formed epsilon martensite phases. However, these martensite phases are rapidly formed at the beginning of the strain, and thus a phenomenon in that the elongation is lowered due to the rapid work hardening is observed. On the other hand, it was confirmed that when the stacking fault energy of the austenite phases calculated by using the corrected formula is more than 37 mJ/m², as a result of investigation with a transmission electron microscope, formation of the martensite phase is not observed after plastic strain. Therefore, it can be seen that the advantageous range of the stacking fault energy of the austenite phases is 19 to 37 mJ/m².

Meanwhile, the lean duplex stainless steel according to the present invention is formed as austenite phases of 45 to 75% and ferrite phases of 25 to 55% by volume fraction.

When the fraction of the austenite phases is less than 45%, an excessive concentration phenomenon of the austenite phase forming elements in the austenite phases occurs during the annealing. Thereby, the austenite phases are sufficiently stabilized to suppress transformation of the strain induced martensite phase which is generated during the strain, and the amount of the austenite phase due to sufficient solid solubility of the alloying elements is increased and thus the tensile strength of the material can be also sufficiently ensured. However, there is a phenomenon in which the ductility is lowered, and the desired sufficient elongation and strength cannot be obtained. Therefore, in view of the high ductility, the fraction of the austenite phase is advantageously 45% or more.

However, when the fraction of the austenite phase exceeds 75%, surface cracks, etc. occur during hot rolling, thereby resulting in deterioration of the hot workability and loss of properties as two-phase structure steel. Therefore, the fraction of the austenite phase is 75% or less.

On the other hand, in the case of the present invention, the range of the critical strain value for strain induced martensite phase formation during the cold processing or the tensile strain is maintained at 0.1 to 0.25.

The amount of critical strain for strain induced martensite phase formation was measured from the inflection point of the stress-strain curve, and this usually refers to the strain value at the time of contributing to the work hardening of the martensite phases in the steel in which the strain induced martensite phase is formed.

In other words, a method of obtaining a critical strain value for strain induced martensite phase formation is described below.

First, after the specimen is taken in accordance with ASTM sub-size standard in parallel with the rolling direction in the cold-rolled annealed material, a tensile test is performed at room temperature (for example, 20 to 25 °C) in a strain rate of 1.0 × 10⁻³/s using the tensile tester until the material is broken. The slope change of the true strain-true stress curve obtained at this time is the work hardening rate. The change in the work hardening rate is closely related to the formation of the strain induced martensite phase. In the case of the work hardening rate, it gradually decreases as the tensile strain progresses after yielding, and then an inflection point is formed at the time point at which the strain induced martensite phase is generated and begins to contribute to the work hardening, i.e. at the critical strain. Then, when the tensile strain progresses due to the strain beyond the inflection point, and at the same time, when the formation of the strain induced martensite phase is increased, the work hardening rate is increased again.

Therefore, the critical strain value is a strain value at a point where the strain induced martensite phase is formed and begins to contribute to work hardening, and refers to the strain value at the point corresponding to the inflection point in the stress-strain curve obtained by the tensile test and mathematically refers to the point at which the second derivative value of the curve becomes zero.

Thus, when the value of the critical strain is less than 0.1, the strain induced martensite phase is easily formed at the time of strain, and the ductility of the material is rapidly lowered due to the rapid work hardening at the beginning of strain. In addition, when the strain induced martensite phase is formed too late, i.e., when the value of the critical strain exceeds 0.25, the elongation rate is lowered due to occurrence of necking which is a local stress concentration by lack of work hardening of the material. Therefore, there is an appropriate range of work hardening rate. Therefore, in the present invention, the range of the critical strain value for strain induced martensite phases formation is 0.1 to 0.25.

In addition, it is very important to control the stability of the austenite phase in the lean duplex stainless steel according to the present invention. Generally, the strain induced martensite phase is a mild phase formed when the unstable austenite phase is strained, and induces work hardening and thus contributes to the increase in the elongation of the steel. In the case of the steel of the present invention, which is a duplex stainless steel consisting of austenite phase and ferrite phase, the stability of the austenite phase can be controlled using the proper distribution of alloying elements. In the present invention, a rapid solidification method is utilized as a method for enabling proper distribution of alloying elements. In the case of rapid solidification, since the time for diffusion occurring in the solid phase is insufficient, the austenite phase and the ferrite phase to be formed are solidified in a non-equilibrium state. When these non-equilibrium solidification phases are subjected to hot-rolling annealing for a short period of time, it is possible to control the stability of the austenite phases sufficiently within a desired range by utilizing the distribution of the generated alloying elements. As a method for achieving this, the alloy was designed so that most of the nitrogen present is segregated on the austenite phases by keeping the content of nitrogen, which has a fast diffusion rate in the solid phase, at a higher content than the normal content.

### Examples

Hereinafter, elongation and corrosion resistance will be described in detail through various embodiments of the lean duplex stainless steel according to the present invention.

The specimens were prepared using a molten steel whose component contents were adjusted as shown in the following table 1. Thereafter, the phase fraction of the material was controlled by proceeding with hot rolling, hot rolling, cold rolling and then cold rolling annealing, and then the elongation and corrosion resistance were measured.

The tensile test specimens were measured by adjusting the tensile strain rate to a rate of 1.0 × 10⁻³/s at room temperature after processing the specimens of ASTM-sub size in parallel to the rolling direction. The following table 1 shows the alloy composition (wt.%) of the test steel.

In addition, the following table 2 below shows the phase fractions of the ferrite phases and the austenite phases of some experimental steels in table 1 measured after annealing heat treatment thereof at 1100 °C.

In addition, table 3 below shows the results of the stacking fault energy values, the differences in Gibbs free energies, the presence or absence of the strain induced martensite phase, the critical strain values, and the elongations for the inventive steels used in the description of the present invention and comparative steels, which were calculated by formula 2 while taking into account the stacking fault energy values, distribution coefficients and phase fraction calculated by formula 1 without considering the distribution coefficient

At this time, the reason for utilizing the Gibbs Free energy difference is that if the difference of the thermodynamic Gibbs free energies calculated when the crystal structure of the phase having the same components is austenite with FCC and when it is martensite with BCC satisfies the condition of ΔG = G^{M} - G^{γ}≤ 0 (Gibbs energy of martensite phase - Gibbs energy of austenite phase), a strain induced martensite phase is formed. Thus, the Gibbs free energy difference and formation of strain induced martensite phase are closely related. For example, it means that when the Gibbs free energy difference (ΔG) is positive, a strain induced martensite phase is not formed, and when the Gibbs free energy difference (ΔG) is negative, a strain induced martensite phase is formed.

In this example, the Gibbs free energies of the austenite phases and the martensite phases were calculated using commercial software FACTsage 6.4 (Thermfact and GTT-Technologies). In particular, in order to calculate the Gibbs free energies, it is first necessary to know the components present in the austenite phase in the steel which is present in two phases of ferrite-austenite phases. The amount of the alloy component present in the austenite phase can be calculated by using the distribution coefficient and the phase fraction shown in the present invention. For example, it is possible to calculate using the component X = X/[K(X) - K(X) × V (γ) + V (γ)] (X: total X component, K(X): distribution coefficient, V(γ): austenite phase fraction) in the austenite phase.

In addition, the presence or absence of formation of the strain induced martensite phase was measured by using a ferrite scope (commercial product) in the crack stretching section before necking during tensile strain

**Table 1:**

| Steel | C | Cr | Ni | Mn | Si | Cu | N | Mo | W |
|---|---|---|---|---|---|---|---|---|---|
| Comp. steel 1 | 0.025 | 21.84 | 2.51 | 1.76 | 0.54 | 0.47 | 0.19 | 0.58 | - |
| Comp. steel 2 | 0.021 | 20.3 | 0.198 | 5.05 | 0.217 | - | 0.102 | - | - |
| Comp. steel 3 | 0.048 | 19.97 | - | 3.02 | 0.201 | 1 | 0.284 | - | - |
| Comp. steel 4 | 0.041 | 23.1 | 0.3 | 3.2 | 2.9 | 0.55 | 0.15 | - | - |
| Comp. steel 5 | 0.003 | 19.8 | 2.4 | 1.7 | 0.3 | 1.6 | 1.28 | - | - |
| Inventive steel 1 | 0.051 | 19.87 | 0.5 | 2.91 | 0.865 | 1 | 0.24 | - | - |
| Inventive steel 2 | 0.05 | 20.12 | 0.205 | 3.03 | 2 | 0.8 | 0.234 | - | - |
| Inventive steel 3 | 0.021 | 19.9 | 0.8 | 3.05 | 0.6 | 1.04 | 0.261 | - | - |
| Inventive steel 4 | 0.052 | 19.7 | 1.01 | 3.1 | 1.2 | 2 | 0.256 | - | - |
| Inventive steel 5 | 0.051 | 21 | 1.02 | 3.02 | 1.1 | 2.03 | 0.254 | - | - |
| Inventive steel 6 | 0.034 | 20 | 1.51 | 3 | 1.95 | 1.5 | 0.251 | - | - |
| Inventive steel 7 | 0.049 | 19.95 | 1.95 | 2.7 | 0.9 | 2.02 | 0.251 | - | - |
| Inventive steel 8 | 0.05 | 19.95 | 1.01 | 2.97 | 2.6 | 1 | 0.235 | - | - |
| Inventive steel 9 | 0.0514 | 19.93 | 1.04 | 2.96 | 1.53 | 1 | 0.32 | - | 0.9 |
| Inventive steel 10 | 0.047 | 21.33 | 1.02 | 3.04 | 1.53 | 1 | 0.23 | - | 0.47 |

**Table 2:**

| Steel | Fraction of ferrite phase | Fraction of austenite phase |
|---|---|---|
| Comp. steel 1 | 51 | 49 |
| Comp. steel 2 | 83 | 17 |
| Comp. steel 3 | 35 | 65 |
| Comp. steel 4 | 54 | 46 |
| Comp. steel 5 | 41 | 59 |
| Inventive steel 1 | 45 | 55 |
| Inventive steel 2 | 37 | 63 |
| Inventive steel 3 | 40 | 60 |
| Inventive steel 4 | 38 | 50 |
| Inventive steel 5 | 28 | 53 |
| Inventive steel 6 | 33 | 67 |
| Inventive steel 7 | 42 | 58 |
| Inventive steel 8 | 47 | 53 |
| Inventive steel 9 | 42 | 58 |
| Inventive steel 10 | 48 | 52 |

**Table 3:**

| Steel | Stacking fault energy (formula 1) without considering distribution (mJ/m²) | Stacking fault energy (formula 2) of austenite phase with considering distribution (mJ/m²) | Gibbs free energy difference | presence or absence of strain induced martensite phase | Critical strain value | Elongation, % |
|---|---|---|---|---|---|---|
| Comp. steel 1 | 29.94 | 33.3 | positive | absence | - | 31 |
| Comp. steel 2 | 15.53 | 33.23 | negative | presence | 0.29 | 38 |
| Comp. steel 3 | 26.21 | 30.87 | negative | presence | 0.07 | 35 |
| Comp. steel 4 | 10.51 | 17.88 | negative | presence | 0.08 | 33 |
| Comp. steel 5 | 31.62 | 37.75 | positive | absence | - | 36 |
| Inventive steel 1 | 17.51 | 23.47 | negative | presence | 0.12 | 52 |
| Inventive steel 2 | 19.33 | 25.60 | negative | presence | 0.143 | 49 |
| Inventive steel 3 | 25.59 | 31.54 | negative | presence | 0.24 | 48 |
| Inventive steel 4 | 24.93 | 33.17 | negative | presence | 0.238 | 53 |
| Inventive steel 5 | 24.20 | 32.03 | negative | presence | 0.219 | 51 |
| Inventive steel 6 | 22.89 | 28.62 | negative | presence | 0.167 | 59 |
| Inventive steel 7 | 27.28 | 33.37 | negative | presence | 0.22 | 57 |
| Inventive steel 8 | 19.33 | 27.40 | negative | presence | 0.182 | 50.5 |
| Inventive steel 9 | 25.49 | 32.78 | negative | presence | 0.24 | 52 |
| Inventive steel 10 | 20.96 | 28.59 | negative | presence | 0.189 | 54 |

In the case of the lean duplex stainless steel, the phase fraction varies depending on the alloy components and the heat treatment temperature.

Thus, table 2 shows the fractions of ferrite phases and austenite phases when heat-treating comparative steels 1 to 5 and inventive steels 1 to 10 at 1100 °C, respectively. It can be seen that in inventive steels 1 to 10, the fractions of the ferrite phases are in the range of about 25 to 55% and the fractions of the austenite phase are in the range of 45 to 75%. Meanwhile, in comparative steel 2, when heat-treating at 1100 °C, the fraction of ferrite phases was 83%, and at this time, the fraction of the austenite phases was 17%. That is, it can be seen that comparative steel 2 is not included in the range of the fractions of the ferrite phase and the austenite phase of the present invention.

In addition, it can be seen that comparative steel 4 has the stacking fault energy of the austenite phase of 17.88 mJ/m² when considering distribution, and thus is not included in the appropriate range of the stacking fault energy (SFE) value of the austenite phase.

On the other hand, fig. 1 is a representative nominal strain-nominal stress comparison curve obtained by the present invention wherein the results of the tensile test after annealing each material at 1100 °C are shown.

In the case of comparative steel 1, strain induced martensite phases were not formed during uniform strain. As a result, there were no strain induced martensite phases that can suppress localized necking due to work hardening during plastic strain, and thus a decrease in elongation was predicted. In fact, the elongation of comparative steel 1 was about 30% which is very inferior.

In addition, in the case of comparative steel 3, it was confirmed that the value of the critical strain for strain induced martensite phase formation at the time of plastic strain is 0.1 or less (inflection point; indicated by an arrow). As a result, it was predicted that the elongation would be lowered due to rapid work hardening in accordance with rapid formation of strain induced martensite phases. In fact, comparative steel 3 is two-phase stainless steel composed of ferrite phase and austenite phase, but the elongation was about 35% which is very inferior.

On the other hand, in the case of the steels of the present invention, it has been shown that when the critical strain range for strain induced martensite phase formation in the stress-strain curve is in the range of 0.1 to 0.25, various values of elongation can be obtained by suitably controlling the rate of formation of the strain induced martensite phase which is formed during processing. That is, when inventive steel 8 and inventive steel 1 are compared, it can be seen that the larger the critical strain for strain induced martensite phase formation, the greater the strain rate. This is to control the transformation of the austenite phases into the strain induced martensite phases during cold working, and the elongation is mostly 45% or more. This result shows that the steel of the present invention has an excellent elongation rate compared to that of the conventional lean duplex stainless steel of comparative steel 1 to be substituted and that the steel of the present invention has an excellent elongation ratio comparable to the elongation of 304 steel to be substituted.

In addition, when the critical strain value is less than 0.1, a sharp reduction of the elongation is caused by the hardening of the material due to the rapid work hardening while the strain induced martensite phase is rapidly formed. In addition, when the critical strain value is more than 0.25, the strain induced martensite phase is formed too late and the local necking of the material due to the strain cannot be suppressed. Therefore, in the case of the lean duplex stainless steel made of the austenite phase-ferrite phase of the present alloy system, when the value of the critical strain for strain induced martensite phase formation becomes 0.1 to 0.25, it is possible to ensure an elongation of 45% or more, which is much better than the elongation of the conventional duplex stainless steel of 30% or less, and to ensure the elongation of 45% or more, which is comparable to 304 steel, under the condition of some strains. Accordingly, the value of the critical strain for strain induced martensite phase formation during the cold processing is 0.1 to 0.25.

In addition, as shown in comparative steel 1 and comparative steel 5 in table 3, it was confirmed that even if the stacking fault energy according to formula 2 is in the range of 19 to 37 mJ/m², the value of the Gibbs free energy at which the martensite phase is formed on the austenite shows a positive value, so that formation of strain induced martensite phase is not observed in the microstructure, observed by the transmission electron microscope, and in this case, it was observed that the elongation is lowered.

Also, as shown in the comparative steel 2 and the comparative steel 3 in table 3, it was observed that even if the value of Gibbs free energy is negative and thus the strain induced martensite phase is formed, the elongation is lowered even when the critical strain value is not in the range of 0.1 to 0.25.

Figs. 2a and 2b show transmission electron microscopic microstructures of comparative steel 1 and inventive steel 1, respectively. In the case of comparative steel 1, as shown in Fig. 2a, it can be seen that strain bands or mechanical twins due to the strain are observed, but the strain induced martensite phase is not observed. In the case of invention steel 1, as shown in Fig. 2b, it can be seen that the strain induced martensite phase is formed at the intersection of the strain bands or the mechanical twins (the strain induced martensite phase is indicated by an arrow).

Fig. 3 is a graph showing the relationship between the elongation and the value of the critical strain for strain induced martensite phase formation. The results of measuring the critical strain for martensite phase formation referring to the stress-strain curve of Fig. 1 are shown in Fig. 3.

Referring to Fig. 3, it can be confirmed that when the values of the critical strain are less than 0.1 or more than 0.25, the elongation of 45% is not ensured, but when the value range of critical strain is 0.1 to 0.25, the elongation of 45% or more can be ensured.

Meanwhile, the lean duplex stainless steels according to the invention can be manufactured by the continuous casting method claimed herein by solving the problem of nitrogen gas generation or emission depending on the difference in nitrogen solubility when solidified from a liquid phase to a solid phase.

First, a method for manufacturing lean duplex stainless steel by a continuous casting method will be described.

Fig. 4 is a schematic view illustrating the manufacturing process of the continuous casting method of the lean duplex stainless steel according to an embodiment of the present invention.

The lean duplex stainless steel according to one embodiment of the present invention is manufactured in a conventional continuous facility 100 in which ladle 110, tundish 120, mold 130, and a plurality of segments 140 are sequentially disposed. Additionally, the rear end of the segment 140 is further provided with a spraying mean 150 for spraying air and cooling water mixed with each other.

In order to manufacture the lean duplex stainless steel by the continuous casting method, first, a molten steel having the above-described alloy components is prepared and moved to the ladle 110, and then temporarily stored in the tundish 120 using a shrouding nozzle 111. At this time, the molten steel temporarily stored in the tundish 120 is maintained at a temperature higher than the theoretical solidification temperature by 10 to 50 °C.

In other words, ΔT (°C.), which is the difference between the temperature of the molten steel and the theoretical solidification temperature in the tundish 120, has a lower limit of 10 °C and an upper limit of 50 °C. The reason is that if ΔT is lower than the lower limit of 10 °C, solidification of the molten steel M can proceed in the tundish 120, thereby causing a problem in continuous casting, and if ΔT exceeds the upper limit of 50 °C, the solidification rate is lowered during solidification and the solidification structure is coarsened, so that solidification cracks in the continuous casting cast slab and linear defects during hot rolling are liable to occur.

Then, in the tundish 120, the molten steel M is injected into the mold 130 using an immersion nozzle 121. At this time, in the mold 130, the molten steel M is passed through the mold 130 to be primarily cooled while maintaining the cooling rate of the molten steel M at 500 to 1500 °C/min.

At this time, when the cooling rate becomes less than 500 °C/min, nitrogen gas generated by the difference in nitrogen solubility due to the initially formed delta ferrite solidification is discharged through the solidified shell of the mold 130, so that coarse nitrogen pinholes are generated and thus a large number of nitrogen pinholes are generated in the continuously cast slab. In addition, coarsening of the initially formed delta ferrite occurs and becomes vulnerable to external stress. Also, when the cooling rate is less than 500 °C/min, the amount of cooling (primary cooling) in the mold 130 and the amount of cooling (secondary cooling) in the segment 140 during the continuous casting are reduced and thereby, during casting, the heat transfer of the cast slab S is delayed, the strength of the cast slab solidified layer is lowered, and the cast slab is bulged, resulting in the deterioration of operation and quality.

In addition, when the cooling rate is controlled to exceed 1500 °C/min, although it is very advantageous from the viewpoint of nitrogen pinhole formation, continuous operation is not possible due to the current limitations of the continuous casting facility, and the time for diffusing the segregation of solute elements remaining between dendrites during continuous casting is shortened, thereby generating surface cracks of the cast slab. There is a problem in that an overlapping phenomenon in which the shell of the cast slab is temporarily broken inside the mold 130 due to such a phenomenon occurs. Therefore, it is necessary to set the cooling rate during the primary cooling in the mold 130 to 500 to 1500 °C/min. The molten steel M, that is, the cast slab S having the solidified shell formed in the casting mold 130 is drawn into the segment 140 and thus cooled secondarily, and at this time it is necessary to spray the cooling water of 0.25 to 0.35 L/kg to the cast slab S. The reason for limiting the spraying amount in the segment 140 in this way is as follows.

If the amount of the sprayed water in the segment 140, i.e., the secondary cooling zone is set to a relatively large value, the solidified structure can be finely formed, but if the amount of the sprayed water exceeds 0.35 L/kg, since the period of time for the segregated impurities to diffuse between the solidified structures in the continuous casting process is reduced, the cast slab is present in a sigma phase, and cracks are generated on the surface of the cast slab. In addition, since not only cracks due to thermal stress but also residual stress is generated on the surface excessively, surface cracks occur during grinding of the cast slab. In addition, when the amount of the sprayed water is less than 0.25 L/kg, there are problems in that the solidification structures become excessive and thus solidification cracks are generated by the sigma phase generated in the grain boundary and in that the strength of the solidification shell of the cast slab is lowered during the continuous casting and the cracks due to bulging of the cast slab is generated.

Therefore, the range of the amount of the sprayed water in the segment 140 is 0.25 to 0.35 L/kg.

In addition, while drawing to the segment 140, a tertiary cooling is performed on the secondarily cooled cast slab S. The tertiary cooling is carried out by spraying the cooling water of 100 to 125 L/kg·min on the entire surface of the cast slab S in the surface temperature range of the cast slab S at 1100 to 1200 °C wherein the air and cooling water are mixed so that the ratio thereof is 1.0 to 1.2 (air/cooling water), while continuing to draw into the segment 140.

The tertiary cooling is controlled so as to ensure a uniform scale on the surface of the cast slab S. The reason for this is that in the case of the lean duplex stainless steel, since the oxidation amount in the heating furnace is very small, the lubrication effect by the scale during the hot rolling is small and thus it is very difficult to reduce surface cracks. Therefore, in order to prevent the reduction of temperature due to the contact between the roll and the steel sheet during rolling and to reduce the frictional force between the roll and the steel sheet to prevent surface cracking, a dense and thick scale should be formed on the surface of the steel sheet and a peeling should not occur easily during rolling. As mentioned above, the reason for limiting the surface temperature of the cast slab S, the amount of the cooling water, and the ratio of the cooling water to air (air/cooling water) is that if the above conditions are not satisfied, a scale having a desired level of thickness (approximately 35*µ*m ± 2*µ*m) is not formed on the surface of the slab S, and the generated scale is not uniformly formed.

Hereinafter, the lean duplex stainless steels having the composition according to the present invention were produced by producing a cast slab while changing the molten steel temperature in the tundish, the cooling rate in the casting mold, and the amount of the sprayed water in the secondary cooling zone as shown in table 4, and the degrees of occurrence of pinholes and cracks on the surface of the cast slab generated therefrom are shown together in table 4. At this time, the occurrence or not of pinholes in the cast slab was measured by grinding the surface of the slab by about 0.5 mm and observing the ground surface.

**Table 4:**

| Material | Degree of overheating of molten steel in tundish (°C) | Cooling rate in mold (°C/min) | Amount of sprayed water in the cooling zone (L/kg) | Degree of occurrence of pinhole | Degree of cracking on surface of continuous casting cast-slab |
|---|---|---|---|---|---|
| Inventive material A | 15 | 1350 | 0.29 | none | none |
| Inventive material B | 20 | 1100 | 0.32 | none | none |
| Inventive material C | 15 | 1100 | 0.27 | none | none |
| Inventive material D | 25 | 850 | 0.29 | none | none |
| Inventive material E | 22 | 550 | 0.3 | none | none |
| Comp. material F | 19 | 1100 | 0.4 | none | serious |
| Comp. material G | 13 | 1100 | 0.2 | none | weak |
| Comp. material H | 20 | 400 | 0.3 | weak | none |
| Comp. material I | 15 | 60 | 0.28 | serious | none |
| Comp. material J | 19 | 40 | 0.29 | serious | none |

As can be seen from table 4, inventive materials A to E which satisfy all of the control conditions of the present invention did not cause pinholes in continuous casting of the cast-slab due to nitrogen and did not cause bulging and defects on the surfaces of the hot-rolled coils.

In addition, since the cooling rates of comparative materials F and G in the mold were within the range of the present invention, pinholes due to nitrogen were not generated in the cast slab. However, in the case of comparative material F, since the amount of the sprayed water was larger than the range of the present invention, no bulging occurred during casting; but thermal stress was severely exerted on the surface of the cast slab, thereby causing occurrence of cracks.

Also, in comparative material G, since the range of the amount of the sprayed water in the secondary cooling zone was less than the range of the present invention, bulging occurred in the cast-slab thereby causing cracks on the surface of the cast-slab. As a result, linear defects occurred on the surface of the hot-rolled coil due to the formation of a local excessive scale during hot rolling.

Also, in comparative materials I and J, the cooling rate in the mold was lower than the range of the present invention, and thus serious pinholes were generated in cast-slab. However, the amount of the sprayed water in the secondary cooling zone is within the scope of the present invention, and thus the surface of the continuous casting cast-slab is good; but a large number of linear defects occurred during the hot rolling due to the pinholes present in the cast-slab.

On the other hand, Fig. 7 is a photograph of the structure of comparative material I and inventive material A produced according to the continuous casting method of the present invention, Fig. 8 is a photograph of surface defects of the comparative material H produced according to the continuous casting method of the present invention and Fig. 9 is a photograph of surface defects of comparative material F produced according to the continuous casting method of the present invention. At this time, Figs. 8 and 9 are photographs of surface defects of the surface of the hot-rolled coils found after the hot rolling of comparative materials H and F.

As can be seen from FIG. 7, it is confirmed that no pinholes were found on the surface of the inventive cast A-slab, but a large number of pinholes were found in comparative material I. Further, as can be seen from Fig. 8, when the surface of the hot-rolled coil after the hot rolling of comparative material H having relatively good occurrence of pinholes are observed, a large number of pinhole-like defects drawn in the rolling direction are observed. In addition, Fig. 9 shows that when the surface of the hot-rolled coil after hot rolling of comparative material F is observed, a large number of crack-like surface defects of cast-slab are observed.

Therefore, it has been confirmed through various embodiments that by properly controlling the cooling rate in the mold and the amount of the sprayed water in the secondary cooling zone during continuous casting according to the present invention, excellent cast-slab quality for the lean duplex stainless steel composed of the austenite phase and the ferrite phase with suppressed occurrence of pinholes, cracking during casting, and bulging can be obtained as well as stable continuous casting operation is possible.

In addition, cast-slab was produced using the lean duplex stainless steel having the composition according to the present invention and subjecting to primary cooling and secondary cooling, while changing the amount of cooling water, the period of spraying time, the air/cooling water ratio, and the surface temperature of cast-slab as shown in table 5, and the thicknesses and the degree of uniformity of the scale obtained therefrom are shown together in Table 5.

**Table 5:**

| Material | Amount of cooling water (L/kg.min) | Period of spraying time (min) | Air/cooling water | Surface temperature of cast-slab (°C) | Thickness of scale (mm) |
|---|---|---|---|---|---|
| Inventive material 1 | 100 | 28 | 1.0 | 1100 | 35 (uniform) |
| Inventive material 2 | 110 | 22 | 1.1 | 1160 | 34 (uniform) |
| Inventive material 3 | 120 | 20 | 1.0 | 1156 | 37 (uniform) |
| Inventive material 4 | 100 | 22 | 1.1 | 1121 | 33 (uniform) |
| Com. material 1 | 50 | 20 | 1.0 | 1111 | 22 (non-uniform) |
| Com. material 2 | 80 | 20 | 1.0 | 1121 | 30 (non-uniform) |
| Com. material 3 | 100 | 20 | 0.5 | 1082 | 10 (non-uniform) |
| Com. material 4 | 100 | 20 | 0.6 | 1198 | 12 (non-uniform) |
| Com. material 5 | 100 | 20 | 0.8 | 1145 | 23 (non-uniform) |
| Com. material 6 | 100 | 15 | 1.0 | 1220 | 22 (non-uniform) |
| Com. material 7 | 100 | 10 | 1.0 | 1230 | 12 (non-uniform) |
| Com. material 8 | 100 | 20 | 1.0 | 932 | 15 (non-uniform) |
| Com. material 9 | 100 | 20 | 1.0 | 1062 | 26 (non-uniform) |

As in inventive materials 1 to 4, it can be seen that when spraying the cooling water for 20 to 30 minutes at a cooling rate of 100 to 120 L/kg · min while keeping the ratio of air/cooling water at 1.0-1.2 at the surface temperature point of cast-slab of 1000 to 1200 °C, the scale becomes very uniform and thick.

However, as in comparative materials 1 and 2, when the cooling water was sprayed at 50 L/kg · min or 80 L/kg · min, the amount of cooling water was insufficient and thus the generation of the oxidized scale was not promoted and a uniform oxidized scale could not be obtained.

Also, as in comparative materials 3 to 5, it was confirmed that when the oxidized scale is investigated while varying the ratio of air to cooling water (air/cooling water), the greater the amount of air, the greater the thickness of the scale layer. Accordingly, in order to form a scale layer having a desired thickness, it is desirable to maintain the ratio of air to cooling water (air/cooling water) to 1.0 or more. However, if the ratio of air exceeds the upper limit of 1.2, a sufficient scale layer can be obtained, but there is a concern that the entire cooling water system will be hindered

As in the comparative materials 6 and 7, when the cooling water is sprayed for the period of spraying time of 15 minutes and 10 minutes, although the temperature of the spraying point of cooling water and the ratio of air/cooling water are in the vicinity of the conditions of the inventive material, a uniform and sufficiently thick scale layer cannot be obtained due to the shortage of the period of spraying time. Therefore, it has been confirmed that in order to obtain a uniform and thick scale layer, the sufficient period of spraying time is required for the slab to react with the air. However, if the period of spraying time of cooling water exceeds a certain period, there is a concern that the cast-slab may become stagnant and the yield may decrease.

In addition, as in the comparative materials 8 and 9, when the cooling water is sprayed at the surface temperature points of cast-slab at 932 and 1062 °C, the thicknesses of the oxidized scales were 15 and 26 µm and the oxidized scales were non-uniform. However, it can be predicted that as the temperature of the cast-slab increases, the formation of the oxidized scale is accelerated and a uniform scale can be obtained. It is also predicted that as the surface temperature of continuous casting cast-slab increases, a uniform scale layer can be obtained.

As described above, in the cooling spraying process after the completion of the continuous casting process, when the optimal amount of cooling water is sprayed at the optimal ratio of cooling water and air at the optimum spraying position, the scale formation can be optimized, the surface quality can be improved, the cost for process for removing defects can be minimized, and thus the added value can be improved.

Next, a method, of manufacturing a lean-duplex stainless steel by strip casting, which is not part of the present invention, will be described:

Fig. 5 is a schematic view showing a manufacturing process of the strip casting method for the lean-duplex stainless steel not forming part of the present invention, and fig. 6 is a photomicrograph of a nitrogen discharge channel formed in the casting roll of the apparatus shown in Figure 5.

The lean duplex stainless steel in this reference method is manufactured in a conventional strip casting facility 200 in which a ladle 210, a tundish 220, a pair of casting rolls 230, inline rollers 260, and winding rolls 270 are sequentially disposed. Additionally, a gas discharge channel 231 is formed on the surface of the casting roll 230.

In order to produce the lean duplex stainless steel by the strip casting method, first, a molten steel M having the above-described alloy components is prepared and moved to the ladle 210, and then temporarily stored in the tundish 220 using a shrouding nozzle 211. Then, the molten steel M is solidified while passing between a pair of casting rolls 230 through an injection nozzle 221 to produce a strip S, and the manufactured strip S is rolled in an inline roller 260 disposed continuously with a casting roll 230 and wound around a winding roll 270.

On the other hand, on the upper side of the casting roll 230, a manifold shield 250 is mounted to prevent the surface of the molten metal from being oxidized by contact with air, and an appropriate gas is added to the inside of the manifold shield 250 to appropriately form an antioxidizing atmosphere.

In this way, the molten steel M is rolled through the inline roller 260 while exiting the roll nip where a pair of casting rolls 230 meet, and then passes through the process such as a heat treatment process and a cold rolling process to form a strip S of 10 mm thickness or less.

One of the most important technical elements in the twin-roll strip casters which directly manufacture the above-mentioned strip S of 10 mm or less is that the molten steel M is provided between a side dam 240 and the inner water-cooled twin-drum rolls 230 rotating at a high speed through the injection nozzle 250 in opposite directions wherein the molten steel M is provided so that the molten steel is rapidly cooled by releasing a large amount of heat through the surface of the water-cooled casting roll 230 and the actual yield is improved without cracking the thin plate of desired thickness.

In the disclosed reference method of producing the highly ductile lean duplex stainless steel, the problems associated with nitrogen exceeding the solubility limit contained in the molten steel, which is the cause of edge cracking and surface cracking, have been solved, and the problem of lowering hot workability due to the nitrogen content has been solved.

That is, by completing the rapid casting while discharging nitrogen exceeding the solubility limit at the time of solidifying the molten steel M through the casting roll 230, and completing the rapid casting by using the inline roller 260, the above-described problem has been solved by producing a thin strip S of about 2 to 5 mm thickness.

Various means can be suggested in order to remove nitrogen exceeding the solubility limit contained in the molten steel M during the strip casting process. As one non-claimed example, in the manufacturing method of a highly ductile duplex stainless steel, the nitrogen discharge channel 231 is formed on the surface of the casting roll 230, thereby discharging nitrogen exceeding the solubility limit in solidifying the molten steel.

The problem of internal porosity due to nitrogen is mostly generated in the process of rapidly cooling the molten steel M while passing between a pair of casting rolls 230.

Therefore, the discharge of nitrogen exceeding the solid solubility limit in the molten steel M must be performed simultaneously with the passage of the molten steel M through the casting roll 230. For this purpose, it is preferable that the gas discharge channel 231 is formed on the surface of the casting roll 230 so that nitrogen can be discharged during casting.

The gas discharge channel 231 is a fine channel to which only the nitrogen gas can be discharged while the molten steel M cannot pass. These gas discharge channels 231 may be formed in the casting roll 230 in various ways and may be formed in the circumferential direction on the surface of the casting roll 230 to guide and discharge the nitrogen gas toward the outside of the casting roll 230 in accordance with the rotation of the casting roll 230.

It is preferable that the gas discharge channel 231 corresponds to a fine channel having a width of 50 to 500 µm and a depth of 50 to 300 µm, and a plurality of gas discharge channels 231 are formed in the circumferential direction of the casting roll 230 wherein the distance between adjacent gas discharge channels 231 is about 100 to 1000 µm.

The shape, structure, and application position of the gas discharge channel 231 may be variously modified as long as the function thereof can be achieved.

On the other hand, when a plurality of such gas discharge channels 231 are formed, the contact area between the casting roll 230 and the molten steel M passing through the casting roll 230 can be reduced and thus in order to prevent this, it is preferable that unevennesses are preferably formed on the surface of the casting roll. These unevennesses have an average size of 15 to 25 µm.

Hereinafter, in order to confirm the effect of nitrogen exceeding the solubility limit in molten steel on the thin plate, a lean duplex stainless steel was produced while changing the composition and casting method of molten steel as shown in the following table 6. Here, comparative example 1 is an example in which molten steel having a specific composition is cast by using a general continuous casting method, comparative example 2 is an example in which molten steel having a specific composition is cast by using a general strip casting (rapid casting) method, and reference examples 1 to 5 are examples in which casting is performed by a strip casting process while discharging nitrogen exceeding the solubility limit in molten steel by using the casting roll having a gas discharge channel formed in a circumferential direction on the outer peripheral surface.

**Table 6:**

| Ex. | C | Si | Mn | Cr | Ni | Cu | N | Casting method | Nitrog en dischar ge | Intern al pore |
|---|---|---|---|---|---|---|---|---|---|---|
| Comp. ex. 1 | 0.05 | 1.35 | 2.8 | 20.3 | 1.06 | 1.0 | 0.23 | continuou s casting | X | O |
| Comp. ex. 2 | 0.05 | 1.35 | 2.8 | 20.3 | 1.06 | 1.0 | 0.23 | rapid casting | X | O |
| Ex. 1 | 0.045 | 1.08 | 3.02 | 19.63 | 0.98 | 0.98 | 0.272 | rapid casting | O | X |
| Ex. 2 | 0.021 | 1.3 | 3.2 | 19.89 | 1.14 | 0.8 | 0.28 | rapid casting | O | X |
| Ex. 3 | 0.031 | 0.6 | 3.0 | 20.02 | 0.9 | 0.7 | 0.24 | rapid casting | O | X |
| Ex. 4 | 0.033 | 1.2 | 3.09 | 20.21 | 0.8 | 0.7 | 0.24 | rapid casting | O | X |
| Ex. 5 | 0.021 | 0.8 | 2.63 | 20.13 | 0.85 | 0.9 | 0.22 | rapid casting | O | X |

As shown in table 6, it was confirmed that in the case of comparative example 1, nitrogen was not discharged during the continuous casting process, and pores were generated inside the cast-slab.

In addition, it was confirmed that in the case of comparative example 2, nitrogen was not discharged during the conventional strip casting process and pores were generated inside the strip.

This is due to the difference in the solubility of nitrogen generated when the molten steel passes through the mold or the casting roll and solidifies

The nitrogen composition of the high ductility duplex stainless steel of the present invention ranges from 1500 to 3200 ppm.

Meanwhile, the process of solidification of the molten steel from the liquid phase to the solid phase proceeds in the order of liquid phase -> liquid phase + delta phase -> delta phase -> delta phase + austenite phase, and when the liquid phase changes into the delta phase, the solubility of nitrogen is about 1164 ppm and thus the solubility difference of about 836 to 1836 ppm occurs. Therefore, some of the supersaturated nitrogen in the liquid phase is gasified during solidification to form various pores in the solidified material and also to form many pores in the solidified shell formed on the surface of the material.

As described above, there are many pores in the actual solidified material. Some of these pores are squeezed during hot rolling, but the non-squeezed pores produce internal defects and develop into a various surface defect form when exposed to the outside during heating in the heating furnace.

On the other hand, it was confirmed that examples 1 to 5 are strip casting processes according to a non-claimed strip casting method in which nitrogen is discharged during the process and pores are not generated in the strip.

Although the invention has been described with reference to the accompanying drawings and the preferred embodiments described above, the present invention is not limited thereto but is limited by the following claim. Therefore, those skilled in the art can variously change and modify the present invention within the scope of the following claim.

### Explanation of symbols

- 100:: Continuous casting equipment, 110: Ladle
- 120:: Tundish, 130: Mold
- 140:: Segment, 150: Spraying means
- 200:: Strip casting facility, 210: Ladle
- 220:: Tundish 230: Casting roll
- 260:: Inline roller 270: Winding roll

## Claims

1. A method of manufacturing a ferritic-austenitic lean duplex stainless steel comprising preparing a molten steel including, by weight, C: 0.08% or less excluding 0%, Si: 0.2 to 3.0%, Mn: 2 to 4%, Cr: 18 to 24%, Ni: 0.2 to 2.5%, Cu: 0.2 to 2.5%, N: 0.15 to 0.32%, optionally at least one of W: 0.1 to 1.0% and Mo: 0.1 to 1.0%, optionally at least one of Ti: 0.001 to 0.1%, Nb: 0.001 to 0.05%, and V: 0.001 to 0.15%, balance Fe and the other unavoidable impurities, continuously casting the stainless steel with additional hot rolling annealing or cold rolling annealing at 900 to 1200°C, wherein the stainless steel is annealing heat treated so that the stacking fault energy (SFE) value of the austenite phase represented by the following Formula 2 is 19 to 37 mJ/m² and the range of the value of the critical strain for strain induced martensite formation is 0.1 to 0.25, wherein the value of the critical strain is measured from the inflection point of the stress-strain curve and obtained by taking a specimen with ASTM sub-size standard in parallel with the rolling direction in cold-rolled annealed material, and a tensile test is performed at 20 to 25°C in a strain rate of 1.0 × 10⁻³/s using the tensile tester until the material is broken: $\begin{matrix}SFE = 25.7 + 1.59 \times Ni / \left[K\left(Ni\right)-K\left(Ni\right)\times V\left(γ\right)+V\left(γ\right)\right] + 0.795 \times Cu / \left[K\left(Cu\right)-K\left(Cu\right)\times V\left(γ\right)+V\left(γ\right)\right] - \\ 0.85 \times Cr / \left[K\left(Cr\right)-K\left(Cr\right)\times V\left(γ\right)+V\left(γ\right)\right] + 0.001 \times {\left(Cr/\left[K\left(Cr\right)-K\left(Cr\right)\times V\left(γ\right)+V\left(γ\right)\right]\right)}^{2} + 38.2 \times {\left(N/\left[\begin{matrix}K \left(N\right) - \\ K \left(N\right) \times V \left(γ\right) + V \left(γ\right)\end{matrix}\right]\right)}^{0.5} \\ - 2.8 \times Si / \left[K\left(Si\right)-K\left(Si\right)\times V\left(γ\right)+V\left(γ\right)\right] - 1.34 \times Mn / \left[\begin{matrix}K \left(Mn\right) - \\ K \left(Mn\right) \times V \left(γ\right) + V \left(γ\right)\end{matrix}\right] \\ + 0.06 \times {\left(Mn/\left[K\left(Mn\right)-K\left(Mn\right)\times V\left(γ\right)+V\left(γ\right)\right]\right)}^{2}\end{matrix}$
wherein the continuous casting includes temporarily storing the molten steel in the tundish while maintaining the temperature of the molten steel at the temperature higher than the theoretical solidification temperature by 10 to 50 °C, primarily cooling the molten steel by injecting the molten steel in the tundish into the mold and passing the molten steel through the mold while maintaining a cooling rate of 500 to 1500 °C/min, secondarily cooling the molten steel having the solidified shell formed by the primary cooling process by spraying cooling water of 0.25 to 0.35 L/Kg on the molten steel having the formed solidified shell while drawing it into a segment and passing through, and tertiary cooling is performed by spraying the cooling water of 100 to 125 L/kg · min on the surface of the cast-slab in the range of the surface temperature of the cast-slab being drawn of 1100 to 1200 °C wherein the cooling water is mixed with air such that the ratio of air to cooling water air/cooling water is 1.0 to 1.2; and
wherein Ni, Cu, Cr, N, Si and Mn refer to the overall content in wt.% of respective constituent elements respectively, and K(x) is represented by the following Formula 3 as the distribution coefficient of respective constituent element (x) measured using Fe-EPMA and FE-TEM, and V(γ) is the fraction of the austenite phase and lies in the range of 0.45 to 0.75: $K \left(x\right) = \left[content of element x in ferrite phase\right] / \left[content of element x in austenite phase\right]$
wherein regarding the K(x), K(Cr) = 1.16, K(Ni) = 0.57, K(Mn) = 0.73, and K(Cu) = 0.64, and K(N) and K(Si) have the following values depending on the content in wt.% of N and Si:
when N is 0.2 to 0.32%, K(N) = 0.15;
when N < 0.2%, K(N) = 0.25;
when Si ≤ 1.5%, K(Si) = 2.76-0.96×Si; and
when Si > 1.5%, K(Si) = 1.4, and
wherein the elongation of the stainless steel is 45% or more, and wherein the lean duplex stainless steel is formed as austenite phases of 45 to 75% and ferrite phases of 25 to 55% by volume fraction, the sum of the austenite and ferrite phases equalling 100%.

## Patentansprüche

1. Verfahren zum Fertigen eines ferritisch-austenitischen Lean-Duplex-Edelstahls, das ein Herstellen einer Stahlschmelze umfasst, die, in Gew.-%, Folgendes beinhaltet: C: 0,08 % oder weniger ausschließlich 0 %, Si: 0,2 bis 3,0 %, Mn: 2 bis 4 %, Cr: 18 bis 24 %, Ni: 0,2 bis 2,5 %, Cu: 0,2 bis 2,5 %, N: 0,15 bis 0,32 %, optional W: 0,1 bis 1,0 % und/oder Mo: 0,1 bis 1,0 %, optional Ti: 0,001 bis 0,1 %, Nb: 0,001 bis 0,05 % und/oder V: 0,001 bis 0,15 %, einen Rest von Fe und die anderen unvermeidbaren Verunreinigungen, Stranggießen des Edelstahls mit zusätzlichem Warmwalzglühen oder Kaltwalzglühen bei 900 bis 1200 °C, wobei der Edelstahl durch Glühen wärmebehandelt wird, sodass der Stapelfehlerenergie(stacking fault energy - SFE)-Wert der Austenitphase, der durch die folgende Formel 2 dargestellt wird, 19 bis 37 mJ/m² beträgt und der Bereich des Wertes der kritischen Dehnung für eine Verformungsmartensitbildung 0,1 bis 0,25 beträgt, wobei der Wert der kritischen Dehnung von dem Wendepunkt der Spannung-Dehnung-Kurve gemessen wird und durch Entnahme einer Probe mit ASTM-Untergrößenstandard parallel zu der Walzrichtung in einem kaltgewalzten, geglühten Material erhalten wird und ein Zugversuch bei 20 bis 25 °C in einer Dehnungsgeschwindigkeit von 1,0 × 10⁻³/s unter Verwendung der Zugprüfmaschine durchgeführt wird, bis das Material bricht: $\begin{matrix}SFE = 25,7 + 1,59 \times Ni / \left[K\left(Ni\right)-K\left(Ni\right)\times V\left(γ\right)+V\left(γ\right)\right] + 0,795 \times Cu / \left[K\left(Cu\right)-K\left(Cu\right)\times V\left(γ\right)+V\left(γ\right)\right] - \\ 0,85 \times Cr / \left[K\left(Cr\right)-K\left(Cr\right)\times V\left(γ\right)+V\left(γ\right)\right] + 0,001 \times {\left(Cr/\left[K\left(Cr\right)-K\left(Cr\right)\times V\left(γ\right)+V\left(γ\right)\right]\right)}^{2} + 38,2 \times {\left(N/\left[\begin{matrix}K \left(N\right) - \\ K \left(N\right) \times V \left(γ\right) + V \left(γ\right)\end{matrix}\right]\right)}^{0.5} \\ - 2,8 \times Si / \left[K\left(Si\right)-K\left(Si\right)\times V\left(γ\right)+V\left(γ\right)\right] - 1,34 \times Mn / \left[\begin{matrix}K \left(Mn\right) - \\ K \left(Mn\right) \times V \left(γ\right) + V \left(γ\right)\end{matrix}\right] \\ + 0,06 \times {\left(Mn/\left[K\left(Mn\right)-K\left(Mn\right)\times V\left(γ\right)+V\left(γ\right)\right]\right)}^{2}\end{matrix}$
wobei das Stranggießen ein vorübergehendes Lagern der Stahlschmelze in dem Zwischenbehälter beinhaltet, während die Temperatur der Stahlschmelze auf der Temperatur höher als die theoretische Erstarrungstemperatur um 10 bis 50 °C gehalten wird, ein primäres Kühlen der Stahlschmelze durch ein Pressen der Stahlschmelze in den Zwischenbehälter in die Form hinein und ein Leiten der Stahlschmelze durch die Form, während eine Abkühlgeschwindigkeit von 500 bis 1500 °C/min gehalten wird, ein sekundäres Kühlen der Stahlschmelze, die die erstarrte Schale aufweist, die durch den primären Kühlvorgang durch ein Sprühen von Kühlwasser von 0,25 bis 0,35 l/kg auf die Stahlschmelze ausgeformt wurde, die die ausgeformte erstarrte Schale aufweist, während sie in ein Segment hineingezogen und durchgeleitet wird, und ein tertiäres Kühlen durch das Sprühen des Kühlwassers von 100 bis 125 l/kg min auf die Oberfläche der stranggegossenen Bramme in dem Bereich der Oberflächentemperatur der stranggegossenen Bramme durchgeführt wird, die von 1100 bis 1200 °C gezogen wird, wobei das Kühlwasser mit Luft derart gemischt wird, dass das Verhältnis von Luft zu Kühlwasserluft/Kühlwasser 1,0 bis 1,2 beträgt; und
wobei sich Ni, Cu, Cr, N, Si und Mn jeweils auf den Gesamtgehalt in Gew.-% der jeweiligen Elementarbestandteile beziehen und K(x) durch die folgende Formel 3 als der Verteilungskoeffizient des jeweiligen Elementarbestandteils (x) dargestellt wird, der unter Verwendung von Fe-EPMA und FE-TEM gemessen wird, und V(γ) der Anteil der Austenitphase ist und in dem Bereich von 0,45 bis 0,75 liegt: $K \left(x\right) = \left[Gehalt von Element x in Ferritphase\right] / \left[\begin{matrix}Gehalt von Element x in \\ Austenitphase\end{matrix}\right]$
wobei bezüglich des K(x), K(Cr) = 1,16, K(Ni) = 0,57, K(Mn) = 0,73 und K(Cu) = 0,64, und K(N) und K(Si) die folgenden Werte abhängig von dem Gehalt in Gew.-% von N und Si aufweisen:
wenn N 0,2 bis 0,32 % beträgt, K(N) = 0,15;
wenn N < 0,2 %, K(N) = 0,25;
wenn Si ≤ 1,5 %, K(Si) = 2,76-0,96×Si; und
wenn Si > 1,5 %, K(Si) = 1,4 und
wobei die Bruchdehnung des Edelstahls 45 % oder mehr beträgt,
und wobei
der Lean-Duplex-Edelstahl als Austenitphasen von 45 bis 75 % und Ferritphasen von 25 bis 55 % Volumenanteil ausgebildet ist, wobei die Summe der Austenit- und der Ferritphasen gleich 100 % beträgt.

## Revendications

1. Procédé de fabrication d'un acier inoxydable duplex pauvre ferritique-austénitique comprenant la préparation d'un acier fondu comportant, en poids, C : 0,08 % ou moins à l'exclusion de 0 %, Si : 0,2 à 3,0 %, Mn : 2 à 4 %, Cr : 18 à 24 %, Ni : 0,2 à 2,5 %, Cu : 0,2 à 2,5 %, N : 0,15 à 0,32 %, éventuellement W : 0,1 à 1,0 % et/ou Mo : 0,1 à 1,0 %, éventuellement Ti : 0,001 à 0,1 % et/ou Nb : 0,001 à 0,05 % et/ou V : 0,001 à 0,15 %, le reste Fe et les autres impuretés inévitables, la coulée en continu de l'acier inoxydable avec un recuit de laminage à chaud ou un recuit de laminage à froid supplémentaire entre 900 et 1200 °C, l'acier inoxydable subissant un recuit traité thermiquement de sorte que la valeur de l'énergie de défaut d'empilement (SFE) de la phase austénite représentée par la formule 2 suivante se trouve entre 19 et 37 mJ/m² et la plage de la valeur de la déformation critique pour la formation de martensite induite par déformation se trouve entre 0,1 et 0,25, la valeur de la déformation critique étant mesurée à partir du point d'inflexion de la courbe contrainte-déformation et obtenue en prenant un échantillon avec la norme de sous-taille ASTM en parallèle au sens de laminage dans un matériau recuit laminé à froid, et un essai de traction étant effectué entre 20 et 25 °C avec une vitesse de déformation de 1,0 × 10⁻³/s à l'aide du dynamomètre jusqu'à le matériel soit cassé : $\begin{matrix}SFE = 25,7 + 1,59 \times Ni / \left[K\left(Ni\right)-K\left(Ni\right)\times V\left(γ\right)+V\left(γ\right)\right] + 0,795 \times \\ Cu / \left[K\left(Cu\right)-K\left(Cu\right)\times V\left(γ\right)+V\left(γ\right)\right] - 0,85 \times Cr / \left[K\left(Cr\right)-K\left(Cr\right)\times V\left(γ\right)+V\left(γ\right)\right] + 0,001 \times \\ {\left(Cr/\left[K\left(Cr\right)-K\left(Cr\right)\times V\left(γ\right)+V\left(γ\right)\right]\right)}^{2} + 38,2 \times {\left(N/\left[K\left(N\right)-K\left(N\right)\times V\left(γ\right)+V\left(γ\right)\right]\right)}^{0.5} - 2,8 \times Si / \\ \left[K\left(Si\right)-K\left(Si\right)\times V\left(γ\right)+V\left(γ\right)\right] - 1,34 \times Mn / \left[K\left(Mn\right)-K\left(Mn\right)\times V\left(γ\right)+V\left(γ\right)\right] + 0,06 \times {\left(Mn/\left[\begin{matrix}K \\ \left(Mn\right) - K \left(Mn\right) \times V \left(γ\right) + V \left(γ\right)\end{matrix}\right]\right)}^{2}\end{matrix}$
la coulée continue comportant le stockage temporaire de l'acier fondu dans le panier de coulée tout en maintenant la température de l'acier fondu à une température supérieure à la température de solidification théorique de 10 à 50 °C, le refroidissement primaire de l'acier fondu en injectant l'acier fondu dans le panier de coulée dans le moule et en faisant passer l'acier fondu à travers le moule tout en maintenant une vitesse de refroidissement de 500 à 1500 °C/min, le refroidissement secondaire de l'acier fondu ayant la coque solidifiée formée par le processus de refroidissement primaire en pulvérisant de l'eau de refroidissement de 0,25 à 0,35 L/kg sur l'acier fondu ayant la coque solidifiée formée tout en l'étirant dans un segment et en passant à travers, et le refroidissement tertiaire étant effectué en pulvérisant l'eau de refroidissement de 100 à 125 L/kg min sur la surface de la brame coulée dans la plage de la température de surface de la brame coulée étirée entre 1100 et 1200 °C, l'eau de refroidissement étant mélangée à de l'air de telle sorte que le rapport de l'air à l'eau de refroidissement air/eau de refroidissement est de 1,0 à 1,2 ; et
Ni, Cu, Cr, N, Si et Mn se référant à la teneur globale en % en poids des éléments constitutifs respectifs respectivement, et K(x) étant représenté par la formule 3 suivante en tant que coefficient de distribution de l'élément constitutif respectif (x) mesuré à l'aide de Fe-EPMA et FE-TEM, et V(γ) étant la fraction de la phase austénite et se situant dans la plage de 0,45 à 0,75 : $K \left(x\right) = \left[teneur en élément x en phase ferrite\right] / \left[\begin{matrix}teneur en élément x en phase \\ austénite\end{matrix}\right]$
en ce qui concerne le K(x), K(Cr) = 1,16, K(Ni) = 0,57, K(Mn) = 0,73 et K(Cu) = 0,64, et K(N) et K(Si) ayant les valeurs suivantes en fonction de la teneur en % en poids de N et Si :
lorsque N est de 0,2 à 0,32 %, K(N) = 0,15 ;
lorsque N < 0,2 %, K(N) = 0,25 ;
lorsque Si ≤ 1,5 %, K(Si) = 2,76 - 0,96 × Si ; et
lorsque Si > 1,5 %, K(Si) = 1,4, et
l'allongement de l'acier inoxydable étant de 45 % ou plus,
et
l'acier inoxydable duplex pauvre étant formé de phases d'austénite de 45 à 75 % et de phases de ferrite de 25 à 55 % en fraction volumique, la somme des phases d'austénite et de ferrite étant égale à 100 %.
